

R. LUCKENBACH,  
APPARATUS FOR CONCENTRATING ORES.  
APPLICATION FILED AUG. 27, 1918.

1,370,601.

Patented Mar. 8, 1921.



Witnesses

Frieda Schleifer

R. M. Abels

Inventor  
Royer Luckenbach  
By Roger Luckenbach  
Attorneys

# UNITED STATES PATENT OFFICE.

ROYER LUCKENBACH, OF PHILADELPHIA, PENNSYLVANIA, ASSIGNOR TO LUCKENBACH PROCESSES, (INC.), OF SAN FRANCISCO, CALIFORNIA, A CORPORATION OF NEVADA.

## APPARATUS FOR CONCENTRATING ORES.

1,370,601.

Specification of Letters Patent.

Patented Mar. 8, 1921.

Application filed August 27, 1918. Serial No. 251,630.

To all whom it may concern:

Be it known that I, ROYER LUCKENBACH, a citizen of the United States, and a resident of Philadelphia, county of Philadelphia, 5 and State of Pennsylvania, have invented a certain new and useful Apparatus for Concentrating Ores, of which the following is a specification.

The invention relates to the concentration of ores by a combined gravity separation and contact process wherein the heavier particles of the pulp comprising mineral values including free metals and chemical compounds of metals are separated from the 10 lighter particles by gravity and the lighter values are separated from the water and gangue of the pulp by adhering to surfaces having a strong preferential affinity for minerals and which will repel the water and gangue which is wetted by the water.

It is well known that metals and heavy mineral substances may be separated from lighter bodies by gravity. In ore concentration this is accomplished by treating 15 finely divided ore with water to form a pulp, agitating the pulp to separate the mineral from the gangue and allowing the latter to float off with the water. It is also known that certain substances have a preferential affinity for minerals and will attract and be attracted by them.

The object of the invention is to provide an apparatus wherein a high percentage of mineral values may be obtained and wherein 20 the percentage of silicious gangue recovered with the values will be considerably reduced, thus producing a recovery practically free of earthy substances.

Other objects of the invention will appear 25 in the following specification and accompanying drawings considered together or separately.

By means of the present invention metallic minerals and their sulfids may be 30 separated from the earthy gangue with which they are associated in nature, and likewise certain non-metallic minerals such as graphite and sulfur may be concentrated.

In addition to separating the mineral 35 values from ores having a flinty or rocky gangue, the invention may be utilized in connection with free metals found in placer or surface mining.

The invention may be carried out in con-

nection with all ores and their mineral constituents which are amenable to treatment by the oil flotation methods at present in use, as well as with other mineral substances which will not be acted on by the mineral selective materials employed in such processes.

The accompanying drawings, forming part of this specification, illustrate one embodiment of the invention. In the drawings like parts in all of the several figures are 65 designated by similar reference characters.

In the drawings—

Figure 1 is a diagrammatic longitudinal section of an apparatus embodying this invention.

Fig. 2 is a transverse section of the same taken on the line 2—2 of Fig. 1.

Fig. 3 is a detail sectional view of a modification.

Fig. 4 is a similar view of another modification.

Fig. 5 is a transverse section of a further modification, the section being taken on the line 5—5 of Fig. 6.

Fig. 6 is a section on the line 6—6 of Fig. 5.

Figs. 7 and 8 are an end and side elevation respectively of a further modification.

In carrying out the invention a tank or casing 1 is provided. The tank comprises 85 a hopper shaped bottom 2 having at its lower extremity a trough 3 having a discharge opening 4 at one end.

Extending longitudinally through the trough 3 is a shaft 3<sup>a</sup> carrying stirring arms 3<sup>b</sup>. The arms are secured to the shaft in spiral arrangement so that material in the trough may be conveyed from the inlet end to the outlet end of the tank. The arms 3<sup>b</sup> are preferably arranged as shown in Fig. 3 95 with side wings 3<sup>c</sup> and end wings 3<sup>d</sup>. By this arrangement the arms in addition to passing the material along the trough will also carry it up and shower it down toward the bottom of the trough thus thoroughly 100 agitating the material. The arms 3<sup>b</sup> are preferably so arranged that the shaft may be driven at a relatively high speed to thoroughly agitate the material but the feed through the trough will be slow. The shaft 105 3<sup>a</sup> may be driven in any manner as by means of a pulley 3<sup>e</sup>.

The tank is provided at the end 5 with a

hopper 6 by means of which ore pulp is delivered to the tank. A diaphragm 7 is arranged transversely across the tank near the inlet end and forms a vestibule 8 for receiving the pulp from the hopper 6. The diaphragm is provided with an opening 9 in axial alinement with the trough 3.

Extending from the diaphragm 7 to the outlet end 10 of the tank and located above the trough 3, is a confined air chamber 11, the sides of which extend into the hopper bottom and to within a short distance of the trough. A pipe or conduit 12 extends longitudinally through the air chamber and is provided with branches 13 each terminating in a sprayer 14. The sprayers are arranged over the center of the trough and are adapted to direct water from the pipe 12 in diverging streams into the trough.

Arranged on each side of the air chamber is a screen comprising two foraminous plates 14 and 15, between which is packed a mattress-like filling 16 of matted or tangled filamentous material. The matted material is not tightly packed in a solid mass between the plates 14 and 15 but is so disposed that numerous tortuous passages are produced which will permit the transport through the mats of fluids and finely divided solid matter in suspension therein.

Extending along each side of the tank above the mats 16 is a launder 17 and each launder discharges the material which has passed through the mats upon a traveling belt 18.

The material of which the mats 16 are composed and the surfaces of the belts 18 are coated with a material having a strong preferential affinity for minerals and certain of their chemical compounds, and which is of such a nature as to repel water and earthy or rocky gangue.

Associated with each belt is a scraper 19 for the purpose of removing the coating from the belt and depositing it in a receptacle 20 from which it may be removed and the mineral values separated from the selective material in any desired manner. Tanks 21 containing selective material are arranged in proximity to the belts and means, such as rollers 22, are provided to recoat the belts.

Such material as will not adhere to the belts as well as such minerals as have not come in contact with the coating are discharged from the belts into hoppers 23, each containing a mat similar in all respects to the mats 14 and 15. From the hoppers 23 the tailings are discharged into chutes 24 by which they will be carried to the dump or the tailings may be directed to other hoppers similar to 23 until all of the mineral values are recovered.

Located at the discharge end of the tank 1 is a sump 4<sup>a</sup>, the upper edge of which is on

a level with the plate 14. A pump 4<sup>b</sup> raises the material from the sump and discharges it into a tank 1<sup>a</sup> similar in all respects to the tank 1 and provided with a water inlet, belts and straining hoppers, in which the operations are repeated.

In the modification illustrated in Fig. 3 the conveyer shaft 25 is tubular and the water for use in the apparatus, instead of being brought in above the conveyer as in Figs. 1 and 2 is discharged from the hollow shaft 25 through perforations 26.

In the modification shown in Fig. 4 an ordinary spiral conveyer 26 is illustrated and the water from a pipe 27 is directed into the bottom of the trough through perforations 28.

In Figs. 5 and 6 is shown a form of apparatus in which the tank 1 is similar to that described except that the mechanical conveyer is omitted and the pulp is transported through the tank by hydraulic action. In the modification the trough 29 is rectangular in cross section, and the bottom thereof is arranged in a series of wave-like undulations. The branches 30 from the pipe 12 are provided with cross heads 31 at their lower extremities. The cross heads are provided with perforations 32 opening toward the outlet 4 of the tank and so positioned relatively to the floor of the trough that water discharged from them will force material on the floor toward the outlet and will agitate lighter materials and force them upward. From the outlet 4 the material will fall into a boot 4<sup>c</sup> from which it may be raised by an elevator 4<sup>d</sup> and deposited on a belt 33 alike in all respects to the belts 18.

In the modification shown in Figs. 7 and 8 is illustrated a form of the device in which the process of the invention may be carried out without the use of mechanical power.

The tank 1<sup>b</sup> is in all respects alike to that shown in Figs. 5 and 6 except that instead of the sump 4<sup>a</sup> a chute 34 is provided. The launders 17 discharge into hoppers 23 as in Fig. 2 and these hoppers discharge into hoppers 35. The material discharged from the chute 34 is received in a tank 1<sup>c</sup> situated on a lower level than the tank 1<sup>b</sup> and wherein the operation is the same as in tank 1<sup>b</sup>.

The operation is as follows:

The pulp, formed of finely divided ore and water, is admitted through the hopper 6 and falls into the trough 3 and is passed therethrough by the conveyer. Water under pressure is admitted through the conduit 12 and sprayed down upon the conveyer and the pulp. The shaft 3<sup>a</sup> is rotated at a high speed and the pulp is thoroughly agitated. The solid particles in the pulp are raised by the blades 3<sup>b</sup> and the heavier particles are slowly passed from the vestibule 8 to the outlet 4.

The water from the sprays will assist in the agitation and thoroughly separate the

lighter from the heavier solid matter. The agitation will cause the fine metallic particles and the gangue to float and as the pulp rises it will be forced through the mats 16 and 17 and the mineral values will adhere to the mineral-selective coating on the entangled material of which the mats are composed. The water and gangue, for which the coating has no affinity, will pass freely 10 through the mats and will be discharged through the launders 17. The air in the air chamber 11 will exert a steady pressure on the surface of the pulp within the chamber and assist in forcing the pulp through the 15 mats.

The discharge from the launders will be carried away by the belts 18 and mineral values contained therein will adhere to the coating and be recovered. The belts will discharge 20 into the hoppers 23 where any remaining values will be retained.

When the mats in the tank and hoppers have taken up all of the mineral of which they are capable, as evidenced by the presence of an abnormal recovery on the belts 25 18 the mats may be recoated by pouring the liquid selective compound into them and when the interstices in the mats are filled by successive layers of the compound and mineral values to cause stoppage of the flow through them the mats may be removed and new ones substituted without serious delay in the operation.

The heavy material escaping from the outlet 35 4 will fall into the sump 4<sup>a</sup>. The water will rise to the height of the launders and be discharged. The material, consisting of heavy minerals and some gangue, in the sump will be raised by the pump 4<sup>b</sup> and discharged 40 into the second tank 1<sup>a</sup> where the operation will be repeated. If desired, untreated pulp may be admitted to the tank 1<sup>a</sup> to supplement the supply from the sump.

The coating and the adhering values may 45 be removed from the material of the mats by a suitable solvent or by heat. When the mats are composed of combustible material such as "excelsior" they, together with the compound, may be burned and the minerals recovered.

In the modifications shown in Figs. 3 and 4 the operation is substantially the same as above but the water being introduced below the mass of the pulp will give a more thorough agitation.

In the modification shown in Figs. 5 and 6 the solid matter in the pulp is fed through the tank by the force of the water alone whereby economy of operation is secured.

The embodiment of the invention illustrated in Figs. 7 and 8 is one in which hydraulic action and gravity only are employed to move the material through the system in carrying out the process. The bottom 65 of the trough is preferably arranged and the

water directed thereto as in Figs. 5 and 6 although it will be understood that the water may be admitted as in Figs. 3 or 4 but with the openings 26 or 28 inclined toward the outlet in order that the water may be directed in that direction.

The invention is particularly efficient where mineral values in extremely fine form are present. In the working of gold, for example, the concentrator frequently encounters fine gold, or "greasy" gold, or tabular gold, or flour gold, which escapes on the surface of the water and they have never been able to overcome that flotation tendency. Even the cyanid-plant operator has often 75 encountered a high-grade floating scum which he never could entirely abolish.

When ore is pulverized so that it may pass through an 80 mesh screen, 75% of it is fine enough to pass a screen of more than 100 80 mesh. When ground to 60, 50% is over 100. It is this extremely fine ore, including gangue as well as values, which has a tendency to float, not only in the amalgamation and cyanid processes but the fine flour-like gangue 90 will float upon the water of the oil flotation process and be recovered with the concentrates. The rocky constituent of the ore being naturally more friable than the mineral will predominate in the flour-like ore and 95 by the process of the present invention such gangue will float through the interstices in the mats while the minerals entrained therewith will adhere to the coating on the matted material.

Instead of introducing ore pulp into the tank the finely divided ore in a dry state may be introduced and the pulp may be formed in the tank by mixing the water from the conduit 12 with the ore.

In accordance with the provisions of the patent statutes, the principle of the invention is described, together with the apparatus which is now considered to represent the best embodiment thereof; but it is desired to have it understood that the apparatus shown is merely illustrative and that the invention may be carried out in other ways.

Having now described the invention what is claimed as new and desired to be secured by Letters Patent of the United States is:—

1. An apparatus for concentrating ore, which comprises a receptacle for the reception of ore pulp, means for agitating the pulp whereby the heavier particles of the ore are separated from the lighter particles by gravity, a porous body comprising material to which mineral values will adhere for intercepting the mineral values in the lighter particles of the ore and separating them from the water and gangue of the pulp, and means for exerting air pressure on the pulp for forcing the same through the porous body.

2. An apparatus for concentrating ore,

which comprises a receptacle for the reception of ore pulp, means for agitating the pulp whereby the heavier particles of the ore are separated from the lighter particles by gravity, a body of tangled elements comprising material to which mineral values will adhere for intercepting the mineral values in the lighter particles of the ore and separating them from the water and gangue of the pulp, and means within the receptacle for exerting air pressure on the pulp to force the same through the body of tangled elements.

3. An apparatus for concentrating ore, which comprises a receptacle for the reception of ore pulp, means for agitating the pulp whereby the heavier particles of the ore are separated from the lighter particles by gravity, means for transporting the heavier particles through the receptacle, a screen, and means for exerting air pressure on a portion of the surface of the pulp for forcing the pulp through the screen whereby the mineral values in the lighter particles of the ore will be intercepted and separated from the water and gangue of the pulp.

4. An apparatus for concentrating ore, which comprises a receptacle for the reception of ore pulp, means for agitating the pulp whereby the heavier particles of the ore are separated from the lighter particles by gravity, a conveyer for transporting the heavier particles through the receptacle, a screen, and an air chamber in communication with the pulp whereby air pressure will be applied to the pulp for forcing the pulp through the screen whereby the mineral values in the lighter particles of the ore will be intercepted and separated from the water and gangue of the pulp.

5. An apparatus for concentrating ore, which comprises a receptacle for the reception of ore pulp, means for agitating the pulp whereby the heavier particles of the ore are separated from the lighter particles by gravity, a screen, an air chamber within which air is compressed by the pulp for forcing the pulp through the screen whereby the mineral values in the lighter particles of the ore will be intercepted and separated from the water and gangue of the pulp, and

means for removing the water and gangue from the receptacle.

6. An apparatus for concentrating ore, which comprises a receptacle, means for introducing finely divided ore into the receptacle, means for adding a fluid to the ore whereby the heavier ore particles will be separated from the lighter ore particles by gravity, means for removing the heavier particles from the receptacle, a screen comprising filamentous elements coated with a material to which mineral values will adhere, an air chamber extending the entire length of the receptacle, the walls of said chamber extending below the surface of the pulp whereby the air within the chamber will force mineral values in the floating ore through said screen whereby values will adhere to the material, and means for discharging the water and gangue from the receptacle.

7. An apparatus for concentrating ore, which comprises a receptacle, means for introducing finely divided ore into the receptacle, means for adding water to the ore and means for agitating the pulp thus formed whereby the heavier ore particles will be separated from the lighter ore particles and the water by gravity, means for removing the heavier particles from the lighter by gravity, there being an air chamber within the receptacle and extending from end to end thereof, a screen of material to which mineral particles will adhere and to which water and gangue will not adhere on each side of the air chamber and interposed between the air chamber and the walls of the receptacle, the upper surfaces of the screens being open to atmospheric pressure, the walls of the air chamber extending below the surface of the pulp whereby air compressed in the chamber will act to force the water and particles floating therein upward through the screens.

This specification signed and witnessed this 5th day of July, 1918.

ROYER LUCKENBACH.

Witnesses:

JAMES F. COLEMAN,  
A. E. RENTON.